

# UNITED STATES PATENT OFFICE.

ALLEN B. NORTON, OF CLEVELAND, OHIO, ASSIGNOR TO THE ALUMINUM CASTINGS COMPANY, OF CLEVELAND, OHIO, A CORPORATION OF OHIO.

## PROCESS OF TREATING CASTINGS.

1,384,033.

Specification of Letters Patent. Patented July 5, 1921.

No Drawing. Application filed August 5, 1918, Serial No. 248,277. Renewed April 11, 1921. Serial No. 460,518.

To all whom it may concern:

Be it known that I, ALLEN B. NORTON, a citizen of the United States, residing at Cleveland, in the county of Cuyahoga and State of Ohio, have invented a certain new and useful Process of Treating Castings, of which the following is a specification.

This invention relates to an improved process of treating porous castings for the purpose of rendering them impervious to fluids and especially to liquids. While, in certain of its broader aspects, the invention is not limited to the treatment of castings of any particular material, it has been devised especially for the treatment of castings made of aluminum or aluminum alloys.

One of the objects of the invention is the provision of a process of treating porous castings to render them leak proof, by which process reagents are caused to enter the pores of the casting and therein to bring about a chemical reaction with the resultant formation of a compound having sufficient bulk to stop the pores.

Another object of the invention is the provision of a process of treating porous castings to render them leak proof by subjecting the constituent material of the castings to the action of a reagent capable of penetrating the pores of the said material and re-acting chemically therewith to form in the pores a compound having sufficient bulk to effectively stop the pores.

Another object of the invention is the provision of a process of the character last referred to in which the pores of the casting are stopped with material insoluble in water, and preferably also in oil.

Another object of the invention is the provision of a process of the character in question especially adapted for the treatment of porous castings made of aluminum or aluminum alloys.

A further object of the invention is the provision of a process of the character in question which is capable of being carried out in a simple and effective manner and at a very moderate cost.

In the use of castings which serve as containers or retainers of fluids it has been found difficult in many cases to secure cast-

ings which would not prevent more or less leakage of the fluids; and various expedients have been proposed to overcome this difficulty. In particular it has been found difficult to produce castings of aluminum or aluminum alloys entirely free from porosity, rendering the castings more or less pervious to fluids; and since such castings are very extensively used under conditions calling for leak-proof qualities, it has been a pressing problem to devise some method of saving the substantial percentage of castings which would otherwise be rejected on account of porosity that would in no wise diminish the utility of the casting for purely structural purposes. For example, aluminum (or, more strictly speaking aluminum alloy) castings are now extensively used in the production of internal combustion engines, the crank case and manifolds commonly being made of aluminum and, in numerous cases, the cylinder block and even the cylinder head are also cast of this material. Also transmission gear cases and oil and water pump parts used in connection with such engines are usually made of aluminum. In the case of each of these castings, porosity, especially porosity marked enough to permit the passage of liquids, destroys the usefulness of the casting. Thus the crank case must not permit leakage of the lubricating oil with which it is interiorly flooded; the manifolds, especially the intake manifolds must be impervious to gasoline and to air and, in many cases, to water, and the cylinder and cylinder head castings must be impervious to the jacket water. Obviously the gear cases and oil pumps must be impervious to oil and the water pumps to water.

Heretofore, as far as I am aware, there has been no satisfactory method of treating aluminum castings to overcome these difficulties, and this I have sought to accomplish by my present invention.

In the treatment of aluminum castings such as have been referred to by my improved process I provide in a suitable container, *e. g.* a steel or iron tank, a more or less concentrated aqueous solution of sodium acetate to which is added ammonium chloride. A satisfactory solution, for example,

would consist of 100 pounds of commercial sodium acetate and 50 pounds of ammonium chlorid dissolved in water to bring the total volume up to 38 cubic feet. In this solution I immerse the casting or as much thereof as is to be treated—ordinarily the casting is immersed bodily—and the solution is then heated preferably nearly to boiling temperature. The solution can be heated 10 in any suitable manner for example, by means of steam coils immersed therein. This treatment of the casting is continued for a variable period depending upon the concentration of the solution and the degree 15 of the porosity of the casting. With a solution of the strength above indicated, the treatment would continue for eight hours or so in case of slight porosity, up to sixteen or even twenty-four hours where the porosity is greater.

Following this treatment of the castings in the hot solution, the castings are removed and allowed to thoroughly drain. This completes the essential steps of the process and 25 the castings can next be tested for leaks in any suitable manner. Ordinarily, however, I prefer, before testing the treated castings to place them in an oven and subject them to a temperature preferably somewhat above 30 212° F. until the castings are thoroughly dried out.

I have not determined the precise chemical reactions that take place in the carrying out of this process which I have described, 35 but the sodium acetate solution, penetrating the pores of the casting, either directly or with intermediate reactions attacks the aluminum with the ultimate formation of aluminum acetate and the heating, more or less 40 prolonged, results in the transformation of the aluminum acetate to aluminum hydroxid and acetic acid. The insoluble aluminum hydroxid thus formed has substantially greater bulk than the aluminum entering 45 into the combination to form the hydroxid and consequently the latter, formed *in situ* in the pores of the casting, serves effectively to stop the pores and render the casting correspondingly impervious to passage of 50 fluids. It is quite probable that the drying or baking of the castings after treatment in the boiling solution, when such drying or baking is carried out, may act to convert some of the aluminum hydroxid to aluminum 55 oxid in addition to driving off free moisture. In either case, the treatment results in the stopping of the pores as above set forth.

I have not referred to the action of the ammonium chlorid, and I am not at present 60 able to explain its action. However, I believe that it assists the reaction between the sodium acetate and the aluminum because the chlorids more readily attack aluminum than do the acetates. It seems probable that 65 the chlorid assists in getting the aluminum

ion into solution and thus facilitates the reaction between the aluminum and the acetate.

As will readily be understood, the action of the solution on the metal of the castings 70 will be more or less marked according to the strength of the solution, the temperature of the solution, and the length of the treatment. Thus by using a more concentrated solution than that above specified, viz., 20 75 pounds of sodium acetate and 10 pounds of ammonium chlorid per cubic foot of water, I have secured good results from a treatment of eight hours even where the porosity of the castings was marked. The application 80 of heat to the solution during the treatment of the castings especially serves to hasten the reaction of the acetate and the aluminum. It is to be observed also, that the heating of the solution and therefore of the 85 castings tends to expand the pores in the latter and to drive off occluded air so that the solution more readily enters the pores of the metal. If it is desired to do so, the treatment can be carried out in hermetically tight 90 chambers from which the air can be exhausted and which can be subjected to greater than atmospheric pressure, for the purposes, respectively, of facilitating the removal of air occluded in the pores of the 95 casting, and subsequently introducing the solution into the pores. Such uses of vacuum and pressure are well understood in connection with impregnation treatments and need not be described in detail.

With respect to the use of vacuum and pressure, I may state that I have been able to secure satisfactory results without recourse to either vacuum or pressure and accordingly the apparatus necessary for carrying out the process and the process itself are simple, readily understood and mastered by the average workman. Obviously the apparatus is capable of being cheaply produced and maintained and the process lends 100 itself to treatment of castings in quantities.

Obviously the substance formed in the pores in the presence of the aqueous solution must be insoluble in water; it is also insoluble in oils. Consequently the process 11 is well adapted for the treatment of internal combustion engine castings such as have been mentioned above.

While I prefer to subject the castings to the action of a reagent in aqueous solution, 12 as has been set forth, it will of course, be understood that the invention is not limited to the use of a reagent in liquid form. For example, the castings might be introduced into a closed chamber and subjected to the 12 action of a reagent in vapor form, the vapor penetrating the pores of the casting and reacting with the metal thereof to form in the pores substance of sufficient bulk to stop the pores, as set forth in connection with the use 13

of an aqueous solution. In particular the invention contemplates the use of acetate vapors for the treatment of aluminum castings, said vapors being generated as in the 5 well known white lead processes or in any other known way.

Other ways of applying or carrying out the invention will occur to those skilled in such matters.

10. What I claim is:

1. A process of treating porous metallic articles which includes subjecting the article to the action of fluid reagents in a manner to cause the latter to enter the pores of the 15 article, forming by chemical reaction within the said pores a solid compound having sufficient bulk to stop the said pores and heating the article to change the nature of the solid compound. 75
2. A process of treating porous castings which includes subjecting the casting to the action of a reagent in a manner to cause the latter to enter the pores of the casting and therein form with the constituent material 25 of the casting a solid compound having sufficient bulk to stop the said pores. 80
3. A process of treating porous castings which includes subjecting the casting to the action of a fluid in a manner to cause the latter to enter the pores of the casting and therein form with the constituent material 30 of the casting a solid compound having sufficient bulk to stop the said pores. 85
4. A process of treating porous castings which includes subjecting the casting to the action of a reagent in the form of an aqueous solution in a manner to cause the latter to enter the pores of the casting and therein form with the constituent material of the casting a solid compound insoluble in oil 40 and having sufficient bulk to stop the said pores. 90
5. A process of treating porous castings which includes immersing the casting in a chemical solution adapted to enter the pores of the casting and therein form with the constituent material of the casting a solid compound having sufficient bulk to stop said pores, and heating the solution and casting 45 to expand the pores of the latter, drive out from said pores occluded air and cause entrance therein of the solution and to intensify the chemical action of the solution on the casting. 100
6. A process of treating porous castings which includes immersing the casting in a chemical solution adapted to enter the pores of the casting and therein form with the constituent material of the casting a solid 50 compound having sufficient bulk to stop said pores, heating the solution and casting to expand the pores of the latter, drive out from said pores occluded air and cause entrance therein of the solution and to intensify the reaction of the chemical solution 55 105
7. A process of treating porous aluminum castings which consists in subjecting the casting to the action of a reagent including an acetate in a manner to cause said reagent to enter the pores of the casting and therein form with the aluminum a solid compound having sufficient bulk to stop the said pores. 75
8. A process of treating porous aluminum castings which consists in immersing the casting in an alkali acetate solution in a manner to cause said solution to enter the pores of the casting and therein form with the aluminum a solid compound having sufficient bulk to stop the said pores. 80
9. A process of treating porous aluminum castings which includes immersing the casting in a solution of sodium acetate and ammonium chlorid in a manner to cause said solution to enter the pores of the casting and therein form with the aluminum a solid compound having sufficient bulk to stop the said pores. 90
10. A process of treating porous aluminum castings which includes immersing the casting in a hot solution of sodium acetate and ammonium chlorid. 95
11. A process of treating porous aluminum castings which includes immersing the casting in a hot solution of sodium acetate and ammonium chlorid and heating the casting, after its removal from the solution, to drive off water. 100
12. A process of treating porous aluminum castings which includes subjecting the casting to the action of a boiling solution of sodium acetate and ammonium chlorid. 105
13. A process of treating porous aluminum castings which consists in subjecting the casting to the action of a reagent including an acetate in a manner to cause said reagent to enter the pores of the casting and therein form with the aluminum a solid compound having sufficient bulk to stop the said pores, and intensifying the reaction of the acetate and aluminum by the application of heat or otherwise. 110
14. A process of treating porous aluminum castings which consists in subjecting the casting to the action of a solution of acetate in a manner to cause said solution to enter the pores of the casting and therein form with the aluminum a solid compound having sufficient bulk to stop the said pores, and intensifying the reaction of the acetate and aluminum by the application of heat or otherwise. 115
15. A process of treating porous aluminum castings which consists in subjecting the castings to the action of a reagent including an alkali acetate and a halogen compound in a manner to cause said reagent to enter the pores of the casting and therein 120
- 65 130

form with the aluminum a solid compound having sufficient bulk to stop the said pores.

16. A process of treating porous aluminum castings which includes immersing the casting in a solution of an alkali acetate and a halogen compound in a manner to cause said solution to enter the pores of the casting and therein form with the aluminum a

solid compound having sufficient bulk to stop the said pores.

17. As a new article of manufacture an aluminum alloy casting having its pores substantially stopped with alumina.

In testimony whereof, I hereunto affix my signature.

ALLEN B. NORTON.